

No. 895,535.

PATENTED AUG. 11, 1908.

G. H. BENJAMIN.  
METHOD OF CASTING HOLLOW METAL BODIES.  
APPLICATION FILED JUNE 8, 1907.



FIG. 1.



FIG.2.



WITNESSES:  
Frederick A. Blount  
Augusta E. Muir

# UNITED STATES PATENT OFFICE.

GEORGE HILLARD BENJAMIN, OF NEW YORK, N. Y., ASSIGNOR TO THE COE BRASS MANUFACTURING COMPANY, A CORPORATION OF CONNECTICUT.

## METHOD OF CASTING HOLLOW METAL BODIES.

No. 895,535:

Specification of Letters Patent.

Patented Aug. 11, 1908.

Application filed June 6, 1907. Serial No. 377,615.

To all whom it may concern:

Be it known that I, GEORGE HILLARD BENJAMIN, a citizen of the United States, residing at the city, county, and State of New York, have invented a Method of Casting Hollow Metal Bodies, of which the following is a specification.

My invention relates to a method of casting hollow metal bodies, especially such as are formed of a metal or alloy which is freely oxidizable, when at the casting temperature.

Steel and iron have heretofore been cast in a horizontally rotatable mold, and this has been possible, owing to the fact that such metals are not freely oxidizable when at the casting temperature.

Broadly stated, my invention consists in casting the molten material of which the hollow metal body is to be formed into a reducing atmosphere, and while therein subjecting it to the action of centrifugal force.

The accompanying drawings will serve to illustrate one form which the apparatus, employed in carrying out the invention, may take, in which

Figure 1 is a longitudinal section, with the parts in the casting position; Fig. 2 is a similar view with the parts in the position for removing the hollow casting; and Fig. 3 is a vertical transverse section on the line X-X of Fig. 1, looking to the left.

Referring to the drawing: 5 indicates a supporting frame; 6 casting cylinder. This cylinder is supported upon bearings 7, so as to enable it to be swung from the position shown in Fig. 1 to that shown in Fig. 2.

8 indicates a hopper, through which the molten metal is fed into the cylinder 6.

9 indicates a tank, containing a reducing gas, which is connected by a pipe 10 to the interior of the hopper 8 and by a pipe 11 to the interior of the cylinder 6. These pipes are provided with suitable valves 12, 13.

It is essential in an apparatus of the character described that the cylinder have its axis of rotation maintained horizontal and that the rotation be uniform. The cylinder 6 may be rotated in any suitable manner, as by a belt, sprocket gear, worm gear, or otherwise.

In the present drawings, I have shown the rotating means as consisting of a polyphase electric motor 14, the rotor member of which is mounted upon the exterior of the cylin-

der 6 and suitably insulated therefrom both electrically and as to heat.

Obviously, after a casting is formed within the cylinder 6, it is necessary to remove it. Many plans may be adopted, which will at once suggest themselves to engineers. One convenient way is, as shown in the figures, *i. e.*,—to mount the motor 14 and cylinder 6 upon bearings 7, so that the cylinder may be swung in the arc of a circle, and mount the coöperating ends 16, 17, which act as closures for the ends of the cylinder, upon sliding bearings 18, 19. These bearings are connected through a handle 20 and coöperating lever arms 21, 22 and 23, so that simultaneous movement toward or from each other may be given to the bearings and ends.

The apparatus above described, as before stated, is such as may be used. Of course, other apparatus may be used.

The method employed consists in preliminarily charging the interior of the cylinder 6 and the hopper 8 with a reducing gas, such, for instance, as carbon oxid or hydrogen under pressure. I prefer that the pressure should be double that of the atmosphere, *i. e.*,—30 pounds to the square inch. After the cylinder and hopper are charged with gas the cylinder is rotated. In practice, I have found that the speed of rotation of the cylinder will vary anywhere from 900 to 2500 revolutions a minute, depending somewhat upon the temperature at which the molten metal is charged into the cylinder.

As soon as the rotation of the cylinder is effected, and, as before stated, is charged with a reducing gas under pressure, the cover 25 of the hopper is raised and the molten metal or alloy slowly poured into the hopper, the pressure of the gas in the hopper and the cylinder being maintained. The metal flows from the hopper into the cylinder and by centrifugal force is distributed to the inner side of the cylinder, distributing itself uniformly over the entire interior of the cylinder. The pouring is continued until a hollow body has been formed of the required thickness.

During the entire pouring, and for some minutes after the pouring has ceased, the pressure of the reducing gas within the cylinder is maintained. The reducing gas within the cylinder acts firstly to remove the air from the interior of the cylinder; secondly,

to prevent access of air to the interior of the cylinder; thirdly, to effect a chemical combination with any occluded air carried by the heated metal or alloy, and fourthly, to reduce any oxid which may be formed on the metal or alloy in the melting operation or during pouring.

I have found in some cases that in order to obtain the best results, it is preferable to 10 combine two reducing gases, as, for instance, hydrogen and carbon.

As soon as the casting is completed and the metal sufficiently cooled, the gas is shut off and the rotation of the cylinder stopped 15 and the cylinder tilted to the position shown in Fig. 2. Contraction of the casting permits it to be readily slid or pulled out of the cylinder.

In practice I have cast hollow ingots from 20 copper, brass, various alloys, zinc, iron and steel, in all cases obtaining a hollow ingot with solid walls, free from blow holes or occluded air, and which are in condition to be subsequently treated by rolling, drawing, 25 etc., as is usual in the manipulation of such bodies.

The essential feature of novelty is, as before stated, the casting of the hot metal into a non-oxidizing atmosphere and while in 30 such atmosphere subjecting it to centrifugal action to cause metal to assume the shape of a hollow body.

It will be evident to engineers, that the same principle may be applied in the formation 35 of other shapes than tubes, for instance, disks, bodies plain on the interior but having angular surfaces, as for instance, hexagon or octagon tubes, and the like.

Having thus described my invention, I 40 claim:

1. The herein described method of forming hollow metal bodies which comprises the provision of and the maintaining of a reducing atmosphere within a rotating mold, feeding 45 the molten material of which the body is to be formed into said mold, and while therein subjecting it to the action of centrifugal force.

2. The herein described method of forming hollow metal bodies which consists in feeding the molten material of which the body is to be formed, into a hollow mold containing a reducing gas under pressure, and while therein subjecting it to the action of 55 centrifugal force.

3. The herein described method of forming hollow metal bodies which consists in feeding the molten material of which the

body is to be formed, into a tubular rotating mold containing a reducing gas under pressure.

4. The herein described method of forming hollow metal bodies which consists in feeding the molten material of which the body is to be formed, into a tubular body rotating around its horizontal axis, and subjecting said metal body while in said tube to the action of a reducing gas under pressure.

5. The herein described method of forming hollow metal bodies, which comprises the exclusion of atmospheric air from and the provision of and the maintaining of a reducing atmosphere within a rotating mold, feeding the molten material of which the body is to be formed into said mold, and while therein subjecting it to the action of said reducing atmosphere and to the action of centrifugal force.

6. The herein described method of forming hollow metal bodies which comprises the provision of and the maintaining of a reducing atmosphere within a hollow horizontally disposed tubular mold rotated at a high speed, feeding the molten material of which the body is to be formed into said mold, and subjecting said material while in said mold to the action of said reducing atmosphere and to the action of centrifugal force.

7. The herein described method of forming hollow metal bodies which comprises melting to a fluid condition the material of which the body is to be formed, the provision of and the maintaining of a reducing atmosphere within a hollow tube rotated at a high speed, feeding said material gradually into said hollow tube, and while therein subjecting said material to the action of said reducing atmosphere and to the action of centrifugal force.

8. The herein described method of forming hollow metal bodies which comprises the maintained exclusion of atmospheric air from within a hollow tube rotated at a high speed, melting to a fluid condition the material of which the body is to be formed, feeding said material gradually into said hollow tube while continuously excluding the atmospheric air from the interior thereof.

In testimony whereof, I affix my signature, in the presence of two witnesses.

GEORGE HILLARD BENJAMIN.

Witnesses:

FREDERICK A. BLOUNT,  
AUGUSTA E. MUIR.